

# UNITED STATES PATENT OFFICE.

HENRI SCHMID, OF MULHOUSE, GERMANY, ASSIGNOR TO BADISCHE ANILIN & SODA FABRIK,  
OF LUDWIGSHAFEN-ON-THE-RHINE, GERMANY, A CORPORATION.

## PRODUCTION OF BROWN SHADES ON THE FIBER.

No. 863,761.

Specification of Letters Patent.

Patented Aug. 20, 1907.

Application filed October 17, 1905. Serial No. 283,139.

To all whom it may concern:

Be it known that I, HENRI SCHMID, chemist, citizen of the Swiss Republic, residing at Mulhouse, in Alsace, German Empire, have invented new and useful Improvements in the Production of Brown Shades on the Fiber, of which the following is a specification.

Attempts to produce brown shades by the oxidation of paraphenylenediamin on the fiber in a manner similar to that in which anilin black is produced, have hitherto met with no technical success, because, when the hydrochlorid is oxidized by means of a chlorate and an oxygen carrier, in particular a vanadium salt, shades are obtained which are not fast and the fiber is greatly corroded and weakened.

15 I have now discovered that excellent results can be obtained if, when making use of para-phenylene-diamin hydrochlorid, a great part, or the whole, of the hydrochloric acid be neutralized, which may be done for instance by means of sodium acetate, or of sodium formate, or of alkali. Instead of starting with para-phenylene-diamin hydrochlorid and then neutralizing the mineral acid, of course the free base itself may be employed. In each case, it is advantageous to add some ammonium chlorid to the bath.

25 When producing anilin black according to the method of Prudhomme potassium ferrocyanid is added to the bath in order to prevent oxidation taking place before it is desirable, this process, however, cannot be followed in the production of brown by the oxidation of 30 para-phenylene-diamin, because potassium ferrocyanid causes the diamin to be precipitated from its solutions. I have discovered that, by the addition of small quantities of such compounds as hydrosulfite NF, or rongalite C, or even a bisulfite, the bath is decolorized and remains for a long time colorless, or almost colorless; further, by the addition of a glycerin-tartar-emetic solution to the bath, the stability thereof is increased still further as is also that of the material which is padded with the bath so prepared.

40 The vanadium salt should be added shortly before the bath is to be used, and only such amount of the bath should be prepared at one time as can be used within a short period. Instead of adding a vanadium salt to the bath, the material can be treated first with a vanadium compound, such for instance as vanadium ferrocyanid, and can then be treated with the bath containing the phenylene-diamin. The material, after being padded, or otherwise treated, with the bath, should be dried rapidly without being heated too strongly, and then can 45 be steamed (in a Mather-Platt apparatus for example), if a uniform shade be desired. A full brown shade, which is fast to washing, can thus be obtained without corrosion or weakening of the fiber.

In order to produce variegated effects, the treated 50 material can be printed with a reducing paste contain-

ing a sulfite, or a bisulfite, or a hydrosulfite, or similar body, for instance, by printing on to the treated and dried material a paste containing potassium sulfite, sodium acetate and hydrosulfite NF, and then steaming, a pure white on a full brown background can be obtained. If it be desired, however, to produce colored effects, there can be mixed with the reducing paste a basic dye which is stable against the action of hydrosulfite and which can be fixed by means of tannin with the addition of such a body as sodium acetate, or chalk. 60 In this case the procedure may be the same as that employed when producing colored effects on material dyed with an azo coloring matter, except that the paste should contain less reducing matter. The usual precautions employed when producing colored discharges 65 can also be followed here, for instance, phenol, or anilin, may be added to the paste.

In carrying out my invention, a homologue or an isomer of para-phenylene-diamin can be employed instead of para-phenylene-diamin.

75 The following is an example of the preparation of a bath in accordance with my invention, but my invention is not limited to this example. Dissolve twenty (20) grams of para-phenylene-diamin in two hundred and fifty (250) cubic centimeters of hot water, add four hundred and fifty (450) cubic centimeters of cold water, and then one gram and a half (1.5) of rongalite C, and solutions of twenty (20) grams each of sodium chlorate and ammonium chlorid, each in fifty (50) cubic centimeters of water. Then add from thirty (30) to forty (40) 80 cubic centimeters of "glycerin-tartar-emetic" solution and add cold water to make up the whole to one (1) liter. Then add fifteen (15) milligrams of ammonium vanadate. The glycerin-tartar-emetic solution can be prepared by dissolving forty (40) grams of tartar emetic 85 in six hundred and twenty (620) cubic centimeters of hot water and three hundred and forty (340) grams of glycerin.

Now what I claim is:

1. The process for the production of brown shades on 95 the fiber by applying to the material a hereinbefore defined phenylenediamin body, and less than one equivalent of mineral acid for each equivalent of phenylenediamin body employed, and a chlorate and a vanadium compound and then causing the oxidation of the phenylenediamin body substantially as described.

2. The process for the production of brown shades on 100 the fiber by applying to the material a mixture containing a para-phenylene-diamin body and less than one equivalent of mineral acid for each equivalent of para-phenylene-diamin body employed and a chlorate and also a vanadium compound, then drying the material and subjecting it to the action of steam.

3. The process for the production of brown shades with 105 discharge effects on the fiber by applying to the material a mixture containing a para-phenylene-diamin body and less than one equivalent of mineral acid for each equivalent of para-phenylene-diamin body employed and a chlorate

and also a vanadium compound, then drying the material, printing it with a paste containing a reducing agent and then subjecting it to the action of steam.

4. The process for the production of brown shades with discharge effects on the fiber by applying to the material a mixture containing a para-phenylene-diamin body and less than one equivalent of mineral acid for each equivalent of para-phenylene-diamin body employed, a glycerin-tartar-emetic solution and a chlorate and also a vanadium compound, then drying the material, printing it with a paste containing a reducing agent and then subjecting it to the action of steam.

5. The process for the production of brown shades with discharge effects on the fiber by applying to the material

a mixture containing a para-phenylene-diamin body and less than one equivalent of mineral acid for each equivalent of para-phenylene-diamin body employed, a glycerin-tartar-emetic solution and a chlorate and also a vanadium compound, then drying the material, printing it with a paste containing a reducing agent and a coloring matter and then subjecting it to the action of steam.

In testimony whereof I have hereunto set my hand in the presence of two subscribing witnesses.

HENRI SCHMID.

Witnesses:

GERT. E. LIEFELD,  
WILH. GOHRIG.